

Aug. 3, 1954

P. L. SCHERESCHEWSKY

2,685,506

PROCESS FOR THE PRODUCTION OF ZINC METAL

Filed June 20, 1951



*Fig. 2.*



INVENTOR

Philippe L. Schereschewsky,

Flocks and Simon

ATTORNEYS

## UNITED STATES PATENT OFFICE

2,685,506

PROCESS FOR THE PRODUCTION OF  
ZINC METAL

Philippe L. Schereschewsky, Washington, D. C.

Application June 20, 1951, Serial No. 232,608

9 Claims. (Cl. 75—87)

1

The present invention relates to a process for the production of zinc metal.

More particularly the present invention relates to a process for obtaining pure zinc from a zinc ore or zinc-bearing material wherein the zinc is largely in the form of zinc oxide.

Although it has previously been proposed to treat zinc bearing materials with reducing gases or, in the alternative, by reducing the molten zinc bearing material with a layer of coke at the surface, in general these prior processes have been characterized by relatively low yield and in some instances by the production of zinc oxide rather than zinc.

The present invention relates to a novel process for the direct production of zinc metal by the reduction of zinc oxide and the volatilization of the zinc thus produced in a rapid and economical manner.

It has further been discovered in accordance with the present invention that by blowing a zinc-containing molten medium having a high zinc content, i. e. more than 18%, with a stream of substantially pure carbon monoxide, the molten zinc medium being provided with a thick layer of coke granules on the surface thereof and a copper matte below the medium, a highly efficient process for the continuous reduction and production of zinc metal was effected.

In accordance with the present invention a conventional water-jacket zinc-fuming furnace is charged with a molten zinc-bearing medium capable of remaining fluid at a temperature between 1200° and 1500° C. while bearing a large proportion of zinc in the form of zinc oxide, as for example from 18 to as high as 35% of zinc, preferably between 20 and 25%. In addition to the zinc-bearing material the furnace is also charged with a copper matte, i. e. largely consisting of copper sulphide, which forms the bottom layer and will be effective to concentrate the lead, copper, nickel and silver of the zinc ore being charged to the furnace.

The present invention may be better understood by a reference to the figures of the drawing wherein:

Fig. 1 is a diagrammatic flow sheet illustrating the process of the present invention; and

Fig. 2 is a diagrammatic detail of a modified heating arrangement for the furnace.

Referring to the figures of the drawing, a conventional type of water-cooled furnace is indicated diagrammatically at 10. The furnace is provided with a layer of high zinc-containing slag 11 and a bottom layer of copper matte 12.

2

In starting the furnace preferably the high zinc-containing slag is molten in separate crucible and charged into the furnace. Thereafter the copper matte is added to the surface of the slag and being of a high specific gravity falls to the bottom while mixing intimately with the slag and picking up lead, silver or iron or excess iron impurities. Thereafter a layer of granulated coke is added to the slag, this layer of coke being relatively thick, i. e. six inches or more, and indicated at 13. The slag is preferably initially heated to a temperature between 1200° and 1500° C. As shown by the arrow 14, the furnace is continuously heated as needed by blowing the same with a mixture of powdered carbon and oxygen. The slag layer is also blown, as indicated by the arrow 15, with a mixture of carbon monoxide and powdered zinc oxide ore. In order to insure proper reduction the slag layer is further blown, as indicated by the arrow 16, with carbon monoxide carrying in suspension powdered carbon. Finally, the matte layer is blown intermittently with small quantities of carbon monoxide as indicated by the arrow 17 in order to insure turbulence and mixing of the matte with the slag.

Passing from the upper end of the furnace 10, as indicated by the arrow 18, is the volatilized zinc and carbon monoxide which is produced in accordance with the following equations:



The carbon monoxide gas carrying the volatilized zinc is led to a suitable condenser, such as the well-known Wheaton-Najarian condenser, indicated at 19, wherein the gas is cooled to a temperature of approximately 500° C. and liquid zinc is produced as indicated by the arrow 20. The carbon monoxide separated in the condenser, as indicated by the arrow 21, goes through a blower 22 and the major portion thereof passes through a regenerative heater 23, as indicated by the arrow 24. In the regenerative heater a portion of the carbon monoxide is burned with air, as indicated by the arrows 25 and 26, to produce heat and to heat the major portion of the carbon monoxide to approximately 1000° C. so that when it is charged into the furnace the carbon monoxide will be at a relative high temperature and will not tend to cause solidification thereof. The turbulence in the furnace and the slag layer thereof, particularly caused by the injection of the relatively hot carbon monoxide,

will cause contact between the slag and the relatively thick layer of coke 13 so that any unreduced zinc oxide will tend to be quickly reduced to zinc and volatilized.

The zinc-bearing medium, or slag, is preferably a basic iron-zinc silicate having the formula  $\text{SiO}_2 \cdot \text{FeO} \cdot \text{ZnO}$  which is capable of retaining its molten, fluid form although containing a high percentage of zinc. This material may be prepared by fusing together iron oxide, silica or silica and lime in order to produce a magma melting at a temperature of approximately  $1200^\circ \text{ C}$ . Thereafter zinc oxide may be added thereto to produce a melt which may contain as high as approximately 35% of zinc and as low as 10% of silica together with a small quantity of lime, the balance being principally ferrous oxide. Preferably, however, a lesser quantity of Zn oxide is added in forming the slag so that the molten slag will be capable of quickly dissolving zinc oxide as added thereto. In addition to blowing the slag with carbon monoxide bearing powdered zinc oxide ore, or in suspension therein as previously pointed out, the molten magma is also blown with carbon monoxide carrying powdered carbon which produces the initial reduction within the body of the slag, further reduction taking place, as heretofore set forth, in the coke layer through which the molten fluid mass is admixed because of the high degree of turbulence. The additional heat necessary may be supplied to the furnace by injecting powdered carbon and oxygen, as indicated at 14, the burning of the carbon and oxygen to carbon monoxide supplying additional heat. Of course if any of the carbon is burned to carbon dioxide this carbon dioxide will be reduced by the excess carbon or by the coke layer so that the output from the furnace is always carbon monoxide and zinc metal, no zinc oxide being volatilized. From time to time some of the zinc-bearing material may be tapped off through the tap indicated diagrammatically at 27 and further quantities of slag components added to the bath to maintain the composition of the molten slag mass. Similarly at rare intervals a tap indicated diagrammatically at 28 is utilized to remove a portion of the matte and matte components may also be added, i. e. copper sulphide. In addition to or in place of burning a portion of the carbon monoxide in the regenerative heater a portion of the carbon monoxide may be taken off through the lead indicated at 29 to a gas turbine indicated at 30 which can drive an A. C. generator, the leads from the generator being indicated diagrammatically at 31. Here again the electricity generated may be utilized to heat the furnace 10 in a conventional manner so as to aid in maintaining the necessary temperature.

Still another method for heating the bath is illustrated in Fig. 2 wherein the carbon monoxide separated from the stream to be recycled instead of being burned in the regenerative heater 23 is fed through a conduit 32 into a radiant tube formed of Carborundum and projecting into the furnace 10. Air is also supplied to the tube 33 through conduit 34.

The following specific example serves to illustrate the invention but is not intended to limit the same:

*Example I*

Into a conventional water-jacketed furnace of approximately 8' x 15', sufficient slag is poured to furnish a layer a foot to a foot and a half in

depth at a temperature of  $1200^\circ$  to  $1300^\circ \text{ C}$ . This slag may be prepared by melting in a crucible or other heating vessel by fusing together iron oxide, silica and a small quantity of lime and thereafter adding zinc oxide so that a molten mass is produced containing 20% of zinc oxide, 10% of silica, a small quantity of lime and the balance iron oxide. Thereafter to the molten slag in the furnace is added sufficient copper matte in liquid form to form a matte layer at the bottom of the furnace of approximately six inches in depth. Finally to the furnace is added sufficient coke of a granular size of from one-fourth to one inch to form a layer of six inches or more on the surface of the liquid slag. Thereafter the furnace is blown with approximately four pounds of carbon monoxide per minute per square foot of bath surface. Part of the carbon monoxide is formed by feeding the furnace with a stream of 20 98% oxygen, i. e. substantially commercially pure oxygen, carrying powdered carbon to furnish sufficient heat to maintain the temperature of the bath at approximately  $1300^\circ \text{ C}$ , or from  $1200^\circ$  to  $1500^\circ \text{ C}$ . To one of the carbon monoxide streams 25 entering the furnace is added additional powdered zinc oxide ore in order to maintain the composition of the bath, and to another carbon monoxide stream entering the bath there is added an excess of carbon. Approximately three additional 30 pounds of carbon monoxide per minute per square foot will be formed as a result of the various reactions so that the final output of gas containing the volatilized zinc will be of the order of seven pounds of carbon monoxide per minute 35 ute per square foot of furnace surface containing approximately three pounds of zinc per minute per square foot of furnace surface. The additional carbon monoxide generated, i. e. the three pounds of carbon monoxide, need not be recycled 40 through the bath and is preferably burned in the preheater 23 to heat the carbon monoxide coming from the condenser through the line 24 from a temperature of  $500^\circ$  to a temperature of  $1000^\circ \text{ C}$ . Preferably the carbon monoxide fed 45 into the furnace is fed through suitable tuyères and at a sufficient rate so as to agitate both the bath and at least a portion of the carbonaceous granular layer above the bath so that the granular coke or other carbonaceous reducing agent will enter into the reaction. Because of this violent agitation a relatively thick layer of coke or other carbonaceous reducing agent may be utilized since the reaction will take place substantially through the entire layer. From time to time additional coke granules may be added to the surface of the bath so as to maintain a layer in excess of six inches thick. The stream of carbon monoxide fed into the matte layer will also result in agitating the same and greatly increase the ability of the matte layer to extract silver and other metals from the zinc oxide ore being fed continuously into the furnace.

I claim:

1. A continuous process for the production of zinc metal from zinc oxide ore which comprises continuously feeding the ore into a molten bath of a zinc-bearing medium capable of remaining fluid at temperatures of between  $1200$  and  $1500^\circ \text{ C}$ . while having a zinc content greater than 18% 60 and having a layer of granular carbonaceous reducing agent on the surface thereof, passing into said bath a high velocity stream of carbon monoxide gas having suspended therein powdered carbon to agitate both said bath and carbonaceous 65 layer and mix the molten bath with the layer,

so as to reduce said zinc oxide ore to zinc metal and produce carbon monoxide, heating said bath to volatilize said zinc metal, condensing said zinc metal and separating the same from the carbon monoxide gas, and recycling at least a part of said carbon monoxide to the molten bath.

2. The process of claim 1 wherein a portion of the carbon monoxide gas produced during the reaction is burned to produce heat which is utilized for heating said bath.

3. The process of claim 1 wherein a portion of the carbon monoxide gas produced is burned and the heat of combustion is utilized to heat the carbon monoxide gas recycled to the bath.

4. The process of claim 1 wherein the bath is heated by the combustion of powdered carbon and oxygen injected thereinto.

5. A continuous process for the production of zinc metal from zinc oxide ore which comprises continuously feeding the ore into a molten bath of a zinc-bearing medium capable of remaining fluid at temperatures of between 1200 and 1500° C. while having a zinc content greater than 18%, a layer of granular carbonaceous reducing agent on the surface thereof and a layer of copper matte 25 below said bath, passing into said bath a high velocity stream of carbon monoxide gas having suspended therein powdered carbon to agitate both said bath and carbonaceous layer and mix the molten bath with the layer, so as to reduce 30

said zinc oxide ore to zinc metal and produce carbon monoxide, and passing into said matte layer a second stream of carbon monoxide gas to admix said matte with said bath and thereby extract metals other than zinc from said ore, heating said bath to volatilize said zinc metal, condensing said zinc metal and separating the same from the carbon monoxide gas and recycling said carbon monoxide to the molten bath.

10 6. The process of claim 1 wherein the layer of granular carbonaceous reducing agent is greater than six inches in thickness.

7. The process of claim 5 wherein the layer of granular carbonaceous reducing agent is greater than six inches in thickness.

8. The process of claim 1 wherein the molten bath is a basic iron-zinc silicate.

15 9. The process of claim 5 wherein the molten bath is a basic iron-zinc silicate.

References Cited in the file of this patent

UNITED STATES PATENTS

| Number    | Name          | Date          |
|-----------|---------------|---------------|
| 701,458   | Armstrong     | June 3, 1902  |
| 2,144,942 | Seguine, Jr.  | Jan. 24, 1939 |
| 2,473,611 | Robson        | June 21, 1949 |
| 2,475,607 | Garbo         | July 12, 1949 |
| 2,493,823 | Morrison      | Jan. 10, 1950 |
| 2,598,743 | Waring et al. | Jan. 3, 1952  |